

Dec. 18, 1928.

1,696,068

R. M. WITHYCOMBE

ARTIFICIAL DENTURE

Filed June 30, 1924

*Fig. 2.*



*Fig. 1.*



Inventor

*Robert M. Withycombe*

By

*Dale L. Potter*

Attorney

## UNITED STATES PATENT OFFICE.

ROBERT MORSE WITHYCOMBE, OF SYDNEY, NEW SOUTH WALES, AUSTRALIA.

## ARTIFICIAL DENTURE.

Application filed June 30, 1924. Serial No. 723,315.

This invention relates to artificial dentures and to a process for making the same.

Broadly, the principle of the invention is carried out by heating or otherwise treating a plate of vulcanite or like substances in a mold, the latter being formed at least in part of a substance having the property of entering into, impregnating, or uniting with the contacting surface material of the vulcanite by a process similar to that of cementation, or case-hardening in metallurgy, so that the denture acquires in the course of the process, an integral surface layer gradually merging from a surface having characteristics imparted to it by the absorption or impregnation of the substance of the mold in maximum degree, and progressively disappearing in the deeper parts of said layer, which substance is chosen with a view to giving the denture those desirable qualities which constitute a patentable improvement over what has previously been known.

In the illustrative embodiment of the invention, which constitutes the subject-matter of the following description, I have chosen to make at least that part of the mold engaging those portions of the vulcanite which will co-act with the mouth tissues, of a composition of matter including certain proportions of copper oxide and sulphur, the same being the subject matter of my companion application Serial No. 722,830 filed June 27, 1924, Patent No. 1,598,668, dated September 7, 1926.

This mold or model may be cast from the usual wax or resinous impression, or from plaster by running in the composition of matter when in molten state.

As has been pointed out in my said companion application, this composition of matter is superior to the plaster of Paris ordinarily used for the model in that it is extremely fluid when cast, therefore filling the minutest interstices in the impression, and that it is non-porous, having a thoroughly impervious and smooth surface which is perpetuated in the vulcanite denture making the latter more satisfactory from a hygienic standpoint than a denture made from a plaster model. Said companion application mentions also other advantages possessed by my novel composition of matter which it does not seem necessary here to enumerate.

In carrying out the process of the present invention, reference may be had to the accompanying drawing in which Figure 1 shows, in perspective, the model for making a palatal denture cast from said novel composition of matter and embedded in the usual way in the lower half of the flask.

Figure 2 is a perspective view of the finished denture.

An illustration of the upper half of the mould, between which, and the lower half the denture is vulcanized, is not considered necessary as this part of the model may be made in the usual manner out of plaster.

When the contents of the flask 1 are subjected to heat and pressure a certain portion of the substance of that model 2 made from the mixture of copper oxide and sulphur is absorbed by the contacting surface of the vulcanite in a way that is not fully understood. Nor is it definitely known whether the change is purely physical, chemical, or both. The re-action effects a decided physical change in the outer surface 3, of the denture 4, it becoming hard, dense, and resilient so that a much thinner plate can be made than formerly, with superior strength and resiliency and therefore less risk of breakage. The surface thus formed is not to be confused with a mere coating, for it is an inseparable, unitary, integral part of the denture, exhibiting no plane of separation. Notwithstanding this, a perfect plane of cleavage is preserved between the model and that part of the substance thereof which is incorporated with the vulcanite so that the model may be broken away from the denture as easily as plaster, in releasing the denture.

The denture made according to the above process may be worn advantageously with the transmuted surface in direct contact with the mouth tissues, as the copper content of the impregnated vulcanite is inherently germicidal, but as the impregnated surface is electrically conductive the denture lends itself readily to a process of electro-plating and may have that surface thereof which comes into contact with the mouth tissues coated with metal in the electrolytic bath.

Although, for the purpose of practical disclosure, the process has been described in the making of a vulcanite denture, it is equally applicable to the treatment of rub-

ber, gum, or like non-conductive substances to give them an electrically conductive surface which can be directly electro-plated.

Having described my invention what I claim as new and desire to secure by Letters Patent, is:

1. A denture comprising a plate of material having the characteristics of vulcanite and formed integrally with a layer composed of sulphur and copper oxide to form a tissue contacting surface of a material superior to vulcanite in hardness and resiliency, which material progressively changes to a state of homogeneity with the vulcanite of the plate in the deeper parts of said layer.

2. A denture comprising a plate of material having the characteristics of vulcanite and formed integrally with a layer composed of sulphur and copper oxide to form a

tissue contacting surface of a material superior to vulcanite in hardness and resiliency and having inherent germicidal properties, which material progressively changes to a state of homogeneity with the vulcanite of the plate in the deeper parts of said layer.

3. The process of making a vulcanized denture which consists in placing vulcanite or the like in a mold, a part of which has a mixture of copper oxide and sulphur in at least the surface thereof, vulcanizing said vulcanite while in contact with said copper containing surface, thereby producing a transmutation in the contacting surface portion of said vulcanite.

In testimony whereof I have hereunto set my hand.

R. MORSE WITHYCOMBE.